

## UNITED STATES PATENT OFFICE

2,138,672

## METHOD FOR PULVERIZING CEMENTED CARBIDES

Frank F. White, Scotia, N. Y., assignor to General Electric Company, a corporation of New York

No Drawing. Application March 30, 1935,  
Serial No. 13,931

8 Claims. (Cl. 83—94)

The present invention relates to sintered hard metal compositions and more particularly to cemented carbides and to a method for treating such carbides whereby they may be easily crushed or pulverized.

A cemented carbide is a sintered composition generally consisting of hard metal carbide particles cemented together by binder metal having a lower melting point than carbide particles.

10 Binder metals commonly employed in cemented carbide compositions are metals of the iron group or combinations of metals of the iron group with other metals such for example as metals of the 6th group of Mendelejeff's Periodic Table of elements and the quantity of such binder material employed usually varies from about 3 to 25% of the weight of the composition although higher percentages of binder material may be employed if desired.

20 Cemented carbides generally are employed as metal cutting tools or as wire drawing or bending dies. When employed as a metal cutting tool the cemented carbide is usually in the form of a small tip which is copper brazed to a supporting 25 steel shank. Since cemented carbide tools are generally quite brittle there is a considerable amount of breakage of such tools. Broken or worn tools heretofore have been salvaged by methods disclosed in the patent to Taylor No.

30 1,895,354, January 24, 1933, and in the patent to Billings No. 1,895,364, January 24, 1933. However, it usually is desirable in salvaging such tools that the pieces of the cemented carbide be reduced to a finely divided or pulverized condition.

35 This can be done, as disclosed in the Taylor patent, by crushing the cemented carbide in a mortar, the crushing being followed by long ball milling. As a rule the cost of the crushing and ball milling is very high and may exceed the cost 40 of providing an equal weight of new ingredients in powdered form.

It is an object of the present invention to provide a method whereby worn or broken cemented carbide compositions may be pulverized in a simple, efficient and inexpensive manner and thereafter pressed into any desired shape and sintered into a hard compact mass.

In carrying out the present invention, pieces of cemented carbide to be salvaged or pulverized 50 are placed, in any desired quantity, in a closed carbon receptacle which for example may be in the form of a tube about 3" x 6" with  $\frac{1}{2}$ " walls. The tube when loaded is heated to a temperature at which the cemented carbide pieces become 55 spongy or bloated. This temperature is main-

tained for a short period of time until the cemented carbide pieces are heated throughout at this temperature after which the pieces are cooled. They then may be crushed easily in any convenient manner, for example in an ore 5 crusher.

When the cemented carbide pieces consist substantially of tungsten carbide and cobalt, the heating temperature employed is preferably above 1600° C. and generally in the neighborhood 10 of 1700° C. and the heating period about 30 seconds. If a temperature lower than 1600° C. is employed there may be some difficulty in crushing the material while if the temperature is materially higher than 1700° C. the cemented carbide when cooled solidifies into a very hard mass. The heat treatment employed is generally carried out in a carbon receptacle so as to provide a carbonaceous atmosphere and to thereby prevent any appreciable reduction in the carbon 20 content of the heat treated material.

The crushed material provided by the present process may be pressed into desired shapes and sintered into a hard tough mass in a manner well known in the art. The invention moreover 25 is not limited to any specific cemented carbide composition but may be applied generally to any composition of that character.

What I claim as new and desire to secure by Letters Patent of the United States, is:

30 1. In a method for pulverizing a hard cemented carbide composition, the steps which comprise heating said cemented carbide in a carbonaceous atmosphere and at a temperature sufficiently high to cause said cemented carbide 35 to assume a spongy condition and thereafter cooling said spongy material.

2. In a method for pulverizing a hard cemented carbide composition, the steps which comprise heating said cemented carbide in a carbonaceous 40 atmosphere and at a temperature sufficiently high to cause said cemented carbide to assume a spongy condition, cooling said spongy material and pulverizing it.

3. In a method for pulverizing hard cemented carbide compositions, the steps which comprise heating said cemented carbide in a carbon tube at a temperature sufficiently high to cause said cemented carbide to assume a spongy condition and then cooling said spongy material.

4. In a method for pulverizing cemented carbide compositions, the steps which comprise heating said cemented carbide in a carbon tube at a temperature sufficiently high to cause said cemented carbide to assume a spongy condition,

cooling said spongy material and then pulverizing it.

5. In a method for pulverizing cemented carbide compositions, the steps which comprise heating said cemented carbide in a closed carbon receptacle at a temperature of about 1600° C. to about 1700° C. and cooling the cemented carbide from that temperature.

6. A method for pulverizing a sintered hard metal composition consisting substantially of hard metal carbide particles cemented together by a binder metal having a lower melting point than the carbide particles which comprises heating said sintered composition in a closed carbon receptacle at a temperature sufficiently high to cause said hard metal composition to become spongy, maintaining said temperature for a short

time, cooling the hard metal composition from that temperature and pulverizing it.

7. The method for pulverizing a sintered hard metal composition containing about 3 to 25% cobalt, the remainder of the composition consisting substantially of tungsten carbide which comprises placing the sintered material in a closed carbon receptacle and heating the receptacle to a temperature in the neighborhood of 1600° C. to 1700° C. for about 30 seconds, cooling the heated material and then pulverizing it.

8. A method for crushing a cemented carbide, said method comprising heating said carbide to a temperature between about 1600° C. and 1700° C., cooling said carbide and then crushing it.

FRANK F. WHITE.